

## UNITED STATES PATENT OFFICE

2,293,470

## FROTH FLOTATION OF SILICEOUS MATERIAL

Harry L. Mead and Ernest J. Maust, Brewster, Fla., assignors to American Cyanamid Company, New York, N. Y., a corporation of Maine

No Drawing. Application March 7, 1940,  
Serial No. 322,771

11 Claims. (Cl. 209—166)

The present invention relates to froth flotation processes for the removal of acidic siliceous gangue from ores containing it.

Attempts have been made in the past to beneficiate ores, particularly non-metallic ores, containing siliceous gangue by froth flotation of the siliceous portion using promoters especially prepared for this purpose. These promoters are in general compounds having a positively charged surface active portion and are usually referred to as "cationic reagents." Typical reagents of this type are quaternary ammonium compounds such as those described in the Lenher U. S. Patent No. 2,132,902, for example

Cetyl trimethylammonium bromide or chloride  
Lauryl trimethyl ammonium chloride or iodide

Cetyl pyridinium bromide

Dimethylbenzyl phenyl ammonium chloride sulfonated in benzyl ring

Beta diethyl amino ethyl oleyl amide acetate  
Beta diethyl amino ethyl oleyl amide hydrochloride

Trimethyl ammonium methyl sulfate or amino oleyl ethylene diamine

Quaternary ammonium compounds containing at least one aliphatic chain with at least eight and not more than twenty carbon atoms in the molecule

Water-soluble or acid solution soluble compounds of amino cellulose such as chitosan acetate

Trimethyl octadecyl ammonium bromide

Trimethyl eicosyl ammonium iodide

Octadecyl pyridinium bromide

Trimethyl octadecyl ammonium chloride

Trimethyl dodecyl ammonium bromide

Trimethyl dodecyl ammonium iodide

Octadecyl beta hydroxyethyl morpholinium bromide

Cetyl beta hydroxyethyl morpholinium bromide

Triethyl octadecyl ammonium bromide

Triethyl cetyl ammonium bromide

Beta stearamidophenyl trimethylammonium methyl sulfate

Octadecyl pyridinium chloride

Octadecyl pyridinium iodide

Octadecyl alpha picolinium bromide

Octadecyl quinolinium bromide

Dodecyl pyridinium bromide

Heptadecylamino hydrochloride

Hexadecylamine hydrochloride

Dodecylamine hydrochloride

and the primary and secondary aliphatic amines having long hydrocarbon chains attached to the nitrogen such as those described in Armour U. S. 55

Patent No. 2,168,840 such as mono- and di-hexyl, octyl and decyl amines and their water-soluble salts and mixed amines butyl dodecyl amine, butyl octadecyl amine and the like.

5 The procedure proposed hitherto using cationic promoters for the flotation of silica give good results with ores which are slime-free and which do not produce slime readily. However, when slime is present, or when the ore readily produces 10 slime, the effect upon flotation of silica is markedly deleterious even upon the use of excessive and prohibitive amounts of the cationic reagent with the result that the flotation of the silica is very incomplete resulting in obtaining a non-floatable 15 product that is unmarketable and non-economical due to the silica it contains.

The most important field of silica flotation at the present time is presented by the Florida pebble phosphate deposits in which finely divided 20 siliceous gangue is intimately associated with the finely divided phosphatic particles, both contained in a matrix wherein the bonding material is made up of phosphatic and aluminous clay. However, up to the present time the use of 25 cationic reagents to effect a silica flotation has not been commercially feasible with phosphatic ores due to the fact that excessive reagent costs resulted or else if the amount of reagent were reduced within commercial limits, the silica removal 30 is not sufficiently complete to produce a high grade phosphate product. The copending applications Serial No. 320,121, filed February 21, 1940, and Serial No. 325,011, filed March 20, 1940, have described a process of silica flotation in 35 which the ore, such as for example, a pebble phosphate ore, is subjected to an extraordinarily complete desliming procedure removing the last trace of existing slime. These procedures have greatly improved the silica removal but encountered difficulties when applied to materials such as certain phosphate rocks which have relatively 40 soft surfaces and which under the conditioning treatment normally preceding froth flotation, tend to disintegrate on the surface to form a small amount of colloidal and semi-colloidal slime. This slime, which is of the material which is not to be floated, appears to be still more deleterious in its effect on silica flotation than the native or original slime which is largely of an 45 aluminous silicate nature, and a very small proportion of this phosphatic slime will exert a greater effect than a corresponding proportion of ordinary argillaceous slime.

According to the present invention we have found that if a thoroughly deslimed ore is ad-

mitted directly to the flotation cell from its desliming operation in a thoroughly deslimed condition that silica can be floated from this ore economically if the reagents are added directly to the flotation cell and both the silica froth and the non-floatable portion are removed from the cell immediately before the non-floatable portion is allowed to produce a slime. In ordinary flotation the ore is generally conditioned in the presence of the reagent before the flotation operation is performed. In the use of the cationic reagents for the flotation of silica this normal conditioning process proves to be detrimental to the flotation operation in that the slime produced from the non-floatable portion so effects the cationic reagent that the silica is inadequately floated, resulting in an inferior non-floated product containing an excessive amount of silica. After the silica has been removed from the non-floatable and slime producing material the silica then may be removed to a cleaning operation or to subsequent handling or flotation steps without injurious effect as the principal source of slime production has been removed. Such a silica froth is then found to be quite stable showing a decided tendency for flocculation of the siliceous particles in the absence of slime.

The flotation of silica with the cationic reagent is so rapid and the effect of slime produced from the non-floatable portion so deleterious that we prefer to remove the silica completely in a single flotation cell. The cationic reagents mentioned heretofore in this specification, and in fact cationic reagents generally, are rapid in their promoter action, and in accordance with the present invention we have found that improved metallurgical results are obtained with them if the time during which the ore is subjected to froth flotation is less than 20 seconds. The normal agitation and attrition produced in the ordinary type of mechanical or pneumatic flotation cell produces a small amount of slime from the non-floatable portion of the ore so that the more rapidly the non-floatable portion is removed from the zone of agitation and attrition the more economically the silica can be floated with smaller amounts of reagent.

The rapidity with which the silica floats is a further feature of the present invention and permits the use of a single cell or a relatively small number of cells in place of a large string, thereby reducing equipment and power costs. To show the rapidity with which slime is formed by agitation within a flotation cell and its effect upon the flotation of silica we show the following table wherein a phosphatic ore of the Florida pebble phosphate type is violently agitated with a cationic active flotation reagent, dioctyl amine.

Table 1

| Feed<br>B. P. L. | Non-float-<br>able<br>B. P. L. | Tail-<br>ing<br>insol. | Silica<br>concen-<br>trate<br>B. P. L. | Ratio | Recov. | Reagents,<br>lbs./t. feed | Seconds<br>agitated<br>prior to<br>aeration |
|------------------|--------------------------------|------------------------|----------------------------------------|-------|--------|---------------------------|---------------------------------------------|
| 27.68            | 76.56                          | 4.30                   | 1.89                                   | 2.90  | 95.4   | .18                       | None                                        |
| 27.73            | 76.87                          | 4.30                   | 1.35                                   | 2.86  | 96.9   | .18                       | 5                                           |
| 27.72            | 76.54                          | 5.35                   | 1.55                                   | 2.87  | 96.2   | .18                       | 10                                          |
| 27.80            | 76.95                          | 5.85                   | 1.11                                   | 2.80  | 97.6   | .18                       | 20                                          |
| 27.59            | 73.96                          | 7.10                   | 1.00                                   | 2.74  | 77.8   | .18                       | 30                                          |

The term "none" in the above table means that air was admitted simultaneously with the start of agitation, i. e., there was no conditioning of the flotation feed before aeration.

In the above table we show that increasing amounts of silica are left behind in the non-floatable portion as the time of agitation is increased and that after 30 seconds of agitation a non-economical phosphate product is obtained from the particular ore treated due to the large amount of silica left with it.

The present invention is not intended to be limited to any particular theory of action. We believe that the rapidity with which the cation active promoter floats silica apparently is due at least in part to the fact that the action of the promoter takes place immediately and leaves no unchanged promoter in the pulp because if an excess of a promoter is used, and the excess recovered from the water associated with the pulp, this excess does not have the same activity.

An example of a flotation test wherein we added a great excess of cationic reagent and attempted to float the silica in a second charge, using the residue solution from the first charge, is shown in Table 2.

Table 2

| Feed                | Silica<br>concen-<br>trate | Phos-<br>phate      | Tailing<br>percent<br>insol. | Cationic reagent                            |
|---------------------|----------------------------|---------------------|------------------------------|---------------------------------------------|
| Grams<br>503<br>501 | Grams<br>265<br>218        | Grams<br>160<br>283 | 1.80<br>18.00                | 3Xnormal amount.<br>Solution of above only. |

The results set out in the above table are easily explained on the above theory that the cationic promoter releases its whole positive charge rapidly to the silica and then retains no further charge so that the excess cannot be recovered and reused. It is practically impossible to determine what goes on at the instant of flotation but the above theory explains the factors set out above easily and we do not know of any other theory of action which would explain the results. Nevertheless it is possible that other factors may be present and for this reason the theory of action is advanced only as a probable explanation without limiting the invention thereto.

Broadly the present invention is not limited to the use of any particular cationic promoter as we have found that the interference of slime with silica flotation appears to be a general characteristic of cationic reagents. In addition to the effect of slime which is the primary feature of the present invention, the prevention of continued contact of the cationic reagent with the flotation material both before and in the course of flotation has a secondary advantage with certain cationic reagents of the aliphatic amine

type, which reagents are very sensitive to chemical changes induced by the presence of air and water which are probably oxidizing and carbonating phenomena although the exact nature has

not been determined. In the case of cationic reagents which are sensitive to air and water, the present invention has the further advantage that no deterioration due to this cause can take place as the period of contact between reagent, air, water and ore is almost instantaneous. The deleterious effect of agitation and aeration of the ore with water and a cationic active flotation reagent, dioctyl amine is shown below in Table 3. 10

Table 3

| Feed<br>B. P. L. | Non-float-<br>able<br>B. P. L. | Tail-<br>ing<br>insol. | Silica<br>concen-<br>trate<br>B. P. L. | Ratio | Recov. | Reagents,<br>lbs./t. feed | Seconds<br>agitated<br>and<br>aerated |
|------------------|--------------------------------|------------------------|----------------------------------------|-------|--------|---------------------------|---------------------------------------|
| 28.21            | 77.41                          | 4.05                   | 2.12                                   | 2.89  | 95.0   | .18                       | None                                  |
| 27.96            | 75.16                          | 5.80                   | 1.57                                   | 2.79  | 96.3   | .18                       | 5                                     |
| 28.31            | 74.99                          | 6.80                   | 1.89                                   | 2.77  | 95.6   | .18                       | 10                                    |
| 28.12            | 74.64                          | 7.00                   | 1.46                                   | 2.74  | 96.9   | .18                       | 15                                    |
| 28.40            | 71.78                          | 11.10                  | 1.57                                   | Out   | Out    | .18                       | 20                                    |
| 27.55            | 63.04                          | 20.88                  | 1.14                                   | Out   | Out    | .18                       | 30                                    |

The term "none" in the above table means that air was admitted simultaneously with the start of agitation and the silica float and phosphate tailing separated immediately, the froth being removed as quickly as it is physically possible. 25

The data in the above table shows that di-

octyl amine is stable unless in contact with air or slime.

The data in the following table show the effect of slime on the floatation of silica from phosphate rock using dioctyl amine as the floatation agent.

Table 5

| Feed<br>B. P. L. | Concentrates |        | Tails<br>B. P. L. | Ratio | Recov. | Amount<br>of slime | Reagent,<br>lbs./t. feed |
|------------------|--------------|--------|-------------------|-------|--------|--------------------|--------------------------|
|                  | B. P. L.     | Insol. |                   |       |        |                    |                          |
| 29.08            | 77.48        | 1.90   | 6.67              | 3.16  | 84.3   | Lb./t.<br>None     | .17                      |
| 28.16            | 38.59        | 50.20  | 3.80              | 1.43  | 95.8   | 1.09               | .17                      |
| 28.64            | 29.71        | 61.75  | 8.56              | 1.05  | 98.8   | 4.35               | .17                      |
| 28.59            | 32.72        | 57.80  | 4.35              | 1.17  | 97.8   | 4.35               | .43                      |

This is an added advantage of the present invention when sensitive cationic reagents are employed and is a feature which is included in a more restricted aspect of the invention.

A comparison of results in Tables 1 and 3 shows that the ore pulp and reagent can be agitated violently for 20 seconds before any deleterious results show up, whereas even 5 seconds of aeration start to show loss of reagent strength.

To show the effect of time alone on the stability of dioctyl amine, an emulsion of the amine

40 It will be noted that even with one pound per ton of slime, or .044%, that the floatation is substantially killed. Even by adding a prohibitive amount of reagent it is impossible to float silica in the presence of slime. These examples show concretely the necessity of floating the silica at once before the floatation cell has time to make slime.

The data in the following table show the effect of increasing the amounts of amine reagent on the floatation of silica.

Table 6

| Feed<br>B. P. L. | Concentrate |        | Tails<br>B. P. L. | Ratio           | Recov. | Reagent,<br>lbs./t.<br>feed | Frother,<br>lbs./t.<br>feed |
|------------------|-------------|--------|-------------------|-----------------|--------|-----------------------------|-----------------------------|
|                  | B. P. L.    | Insol. |                   |                 |        |                             |                             |
| 30.96            | 33.49       | 57.05  | 5.18              | No stable froth |        | .04                         | .05                         |
| 31.05            | 54.49       | 31.50  | 3.34              | No stable froth |        | .09                         | .12                         |
| 31.49            | 69.52       | 12.60  | 2.71              | No stable froth |        | .13                         | .17                         |
| 31.33            | 75.43       | 5.55   | 1.92              | No stable froth |        | .18                         | .24                         |
| 31.65            | 77.57       | 3.65   | 2.38              | 2.57            | 95.4   | .22                         | .29                         |
| 31.63            | 78.11       | 2.50   | 2.16              | 2.58            | 95.7   | .27                         | .36                         |
| 32.24            | 77.79       | 2.65   | 3.04              | 2.56            | 94.3   | .31                         | .41                         |
| 31.93            | 79.30       | 2.40   | 3.56              | 2.67            | 93.0   | .36                         | .48                         |
| 31.71            | 78.75       | 2.05   | 4.21              | 2.71            | 91.6   | .40                         | .53                         |
| 31.43            | 79.08       | 2.15   | 4.87              | 2.79            | 90.2   | .45                         | .60                         |

representing a 40:1 mixture of dioctyl amine solvent and water was prepared. A portion of the fresh emulsion representing .18 lbs./ton of ore was used immediately, to produce a silica float from a phosphate ore by adding directly to the ore pulp during the floatation. A second portion of the emulsified amine was left standing in a closed container for 18 hours and an .18 lb./ton emulsion used in the same manner to produce a silica float. 65

The data is found in the following table.

70 The above tests were made with a typical cation active promoter, dioctyl amine. Similar results are obtained with the other type of cation active promoters such as those described in the opening paragraphs of this specification. We have found that it is not necessary to the present invention to use ionizable compounds as similar results are obtained with amines and with their ionized salts, provided satisfactory dispersion and distribution is effected. The present invention is therefore not intended to be limited in any way

to the use of a cation active promoter which is actually an ionizable compound. The interaction between the surface of the silica and the basic portion of the promoter does not appear to be tied up exclusively with the presence of actual ions. The theory advanced in the Lenher patent referred to above does not appear to be correct as applied to silica flotation, or at least it does not appear to be a necessary factor in the present invention. For while Lenher is quite correct that all of the materials which he describes in his patent and which are ionized are usable as silica promoters, and show improved results when used in accordance with the procedure which forms the subject of the present invention, the improved results obtainable are not limited to these materials but the amines themselves which are in many cases not water-soluble and are not accordingly ionized, behave in precisely the same way. We do not wish to advance any definite theory of action in silica flotation and the present invention is not intended to be limited to any particular theory of the Lenher patent.

From the foregoing examples it will be apparent to those skilled in the art that the flotation of silica can be accomplished almost instantly by the improved process of the present invention, that fewer flotation cells can be employed to produce a higher grade phosphate product and at the same time use a smaller quantity of flotation reagent.

What we claim is:

1. A process for separating by froth flotation a siliceous gangue from an ore containing a portion which is not readily floatable by promoters for silica flotation and which ore produces additional slime under the ordinary agitation and aeration of a froth flotation cell which comprises desliming the feed, introducing the feed into a froth flotation cell, adding a cationic silica flotation promoter directly to the deslimed ore pulp in the froth flotation cell without preliminary conditioning, effecting froth flotation in said cell, removing therefrom a concentrate relatively rich in siliceous gangue, the time during which the ore pulp is subjected to froth flotation being less than twenty seconds.

2. A process for separating by froth flotation a siliceous gangue from an ore containing a portion which is not readily floatable by promoters for silica flotation and which ore produces additional slime under the ordinary agitation and aeration of a froth flotation cell which comprises desliming the feed, introducing the feed into a froth flotation cell, adding a cationic silica flotation promoter which is subject to deterioration in contact with air and water directly to the deslimed ore pulp in the froth flotation cell without preliminary conditioning, effecting froth flotation in said cell, removing therefrom a concentrate relatively rich in siliceous gangue, the time during which the ore pulp is subjected to froth flotation being less than twenty seconds.

3. A process for separating by froth flotation a siliceous gangue from phosphate ore which ore produces additional slime under the ordinary agitation and aeration of a froth flotation cell which comprises desliming the feed, introducing the feed into a froth flotation cell, adding a cationic silica flotation promoter directly to the deslimed ore pulp in the froth flotation cell without preliminary conditioning, effecting froth flotation in said cell, removing therefrom a concentrate relatively rich in siliceous gangue, the time during

which the ore pulp is subjected to froth flotation being less than twenty seconds.

4. A process for separating by froth flotation a siliceous gangue from phosphate ore which ore produces additional slime under the ordinary agitation and aeration of a froth flotation cell which comprises desliming the feed, introducing the feed into a froth flotation cell, adding a cationic silica flotation promoter which is subject to deterioration in contact with air and water directly to the deslimed ore pulp in the froth flotation cell without preliminary conditioning, effecting froth flotation in said cell, removing therefrom a concentrate relatively rich in siliceous gangue, the time during which the ore pulp is subjected to froth flotation being less than twenty seconds.

5. A process for separating by froth flotation a siliceous gangue from an ore containing a portion which is not readily floatable by promoters for silica flotation and which ore produces additional slime under the ordinary agitation and aeration of a froth flotation cell which comprises desliming the feed, introducing the feed into a froth flotation cell, adding a cationic amine silica flotation promoter directly to the deslimed ore pulp in the froth flotation cell without preliminary conditioning, effecting froth flotation in said cell, removing therefrom a concentrate relatively rich in siliceous gangue, the time during which the ore pulp is subjected to froth flotation being less than twenty seconds.

6. A process for separating by froth flotation a siliceous gangue from an ore containing a portion which is not readily floatable by promoters for silica flotation and which ore produces additional slime under the ordinary agitation and aeration of a froth flotation cell which comprises desliming the feed, introducing the feed into a froth flotation cell, adding a silica flotation promoter, diethyl amine, directly to the deslimed froth flotation in said cell, removing therefrom a concentrate relatively rich in siliceous gangue, the time during which the ore pulp is subjected to froth flotation being less than twenty seconds.

7. A process for separating by froth flotation a siliceous gangue from an ore containing a portion which is not readily floatable by promoters for silica flotation and which ore produces additional slime under the ordinary agitation and aeration of a froth flotation cell which comprises desliming the feed, introducing the feed into a froth flotation cell, adding a silica flotation promoter, lauryl amine, directly to the deslimed ore pulp in the froth flotation cell without preliminary conditioning, effecting froth flotation in said cell, removing therefrom a concentrate relatively rich in siliceous gangue, the time during which the ore pulp is subjected to froth flotation being less than twenty seconds.

8. A method according to claim 3 in which the phosphatic ore is Florida pebble phosphate.

9. A method according to claim 4 in which the phosphatic ore is Florida pebble phosphate.

10. A method according to claim 1 in which the flotation is effected in a single rougher cell followed by cleaning of the silica concentrate produced.

11. A method according to claim 3 in which the flotation is effected in a single rougher cell followed by cleaning of the silica concentrate produced.